

July 5, 1960

M. J. SAARIVIRTA

2,943,960

PROCESS FOR MAKING WROUGHT COPPER-TITANIUM ALLOYS

Filed Aug. 27, 1957

2 Sheets-Sheet 1



INVENTOR  
MATTI J. SAARIVIRTA

BY

Kasper T. Serjan  
ATTORNEY

July 5, 1960

M. J. SAARIVIRTA

2,943,960

PROCESS FOR MAKING WROUGHT COPPER-TITANIUM ALLOYS

Filed Aug. 27, 1957

2 Sheets-Sheet 2

T19.3.



T19.4.

INVENTOR  
MATTI J. SAARIVIRTA  
BY  
Kaaper T. Serijan  
ATTORNEY

1

2,943,960

## PROCESS FOR MAKING WROUGHT COPPER-TITANIUM ALLOYS

Matti J. Saarivirta, Plainfield, N.J., assignor to American Metal Climax, Inc., New York, N.Y., a corporation of New York

Filed Aug. 27, 1957, Ser. No. 680,439

4 Claims. (Cl. 148—12.7)

This invention relates to copper base alloys of the age hardenable type and relates more particularly to binary alloys consisting of copper and titanium characterized by markedly improved workability both hot and cold. In one of its aspects, the invention concerns copper-titanium alloys in wrought form possessing excellent tensile strength, improved resistance to softening at elevated temperature, good ductility, moderate electrical conductivity and other desirable properties. In another of its aspects, this invention concerns methods of treatment whereby very high strength wrought alloys are produced in a very practical, efficient and economical manner. The new and novel wrought alloys provide excellent materials for use in the fabrication of springs, electrical contacts, tools and for numerous other applications requiring particularly high strength combined with other desirable properties and characteristics.

It has long been known that age-hardenable copper-titanium alloys may be processed to provide materials of high strength, in some instances resulting in a tensile strength of about 200,000 p.s.i. or even higher depending upon the amount of titanium present in the alloy. In U.S. Patent No. 1,991,162 issued to Kroll, there are disclosed, for example, copper-titanium alloys containing varying amounts of titanium, and in the case of the alloy containing 4% titanium, a tensile strength of 150 kg./mm.<sup>2</sup> (approximately 213,000 p.s.i.) and an elongation of 1% is indicated. To achieve these mechanical properties, however, it was apparently necessary to age the alloy and thereafter subject the aged alloy to cold-stretching.

Although hot and cold working of copper-titanium alloys prior to the aging step has also been heretofore suggested, the resulting wrought alloys, as far as I have been able to determine, possess much lower tensile strength values compared to the wrought alloys produced by cold-stretching the aged material.

As is well known to those skilled in the art, the step of cold-stretching is not readily or conveniently applicable to all forms of the material being processed, and in some instances, the effective use of cold-stretching is entirely impractical if not virtually impossible. Moreover, cold-stretching the aged alloy lowers the resistance of the alloy to softening at elevated temperatures and generally reduces its resistivity toward corrosion.

Although copper-titanium alloys of the type previously reported containing up to 5 or 6% by weight titanium may be subjected to hot and cold working or both, the extent to which these operations may be carried out is limited by the actual workability of these alloys. In the case of hot working, for example, preheated bars subjected to hot rolling fracture severely on the first or second pass involving relatively small reductions in area. At the same time a reduction of more than 50% by hot working is actually required to completely deform the cast crystal structure and this cannot be accomplished with the conventional copper-titanium alloys due to their marked susceptibility to brittleness on hot working.

Extensive cold working of the conventional copper-

2

titanium alloys is likewise precluded due to the tendency of the material to become embrittled rather rapidly especially when the titanium content is about 3% or higher. Thus, the application of cold working to the extent required in conjunction with appropriate heat treatment of the cold worked material to develop a suitable condition conducive to the production of high strength alloys is entirely impractical without resorting to cold-stretching the aged material which procedure, as previously indicated, is of limited applicability as well as being detrimental to other properties of the resulting alloys.

It is a principal object of this invention to provide new and novel wrought copper-titanium alloys possessing excellent strength and other desirable properties without resorting to cold-stretching the previously aged alloy as heretofore required for producing comparable strength.

Another object of this invention is to provide an entirely practicable and commercially applicable process for the treatment of age-hardenable copper-titanium alloys prepared under oxygen-excluding conditions and containing up to the maximum solid solubility of titanium whereby high strength wrought alloys having other desirable properties including improved resistance to softening at elevated temperatures are readily obtained.

Other objects and advantages will become apparent as this specification proceeds.

It has now been discovered that the workability of copper-titanium alloys containing up to the maximum solid solubility amount of titanium is drastically affected by the presence of oxygen in any form in the copper used in making the alloys. More specifically, I have found that when high purity, initially oxygen-free copper is used in making copper-titanium castings under oxygen-excluding conditions and containing an amount of titanium within the maximum solid solubility in such copper, such castings possess markedly improved workability. When these castings are processed into wrought materials such as wires, rods, sheet or in any other desired form employing appropriate working and heating cycles as hereinafter described in detail, materials of excellent tensile strength together with other highly desirable properties are readily obtained. The enhanced workability accounts for many important advantages including (1) eliminating the need for cold stretching the previously age-hardenable alloy for the purpose of providing high tensile strength, (2) making possible the production of extremely high strength wrought copper-titanium alloys by processing steps involving extensive working after solution annealing but before the age hardening treatment which are completely practical and readily adaptable to commercial production while at the same time improving such properties as the resistance to softening of the wrought product at elevated temperatures, and (3) permitting greater reductions which enable more rapid processing while minimizing the number of solution anneals actually required thereby enabling the production of the high tensile strength wrought alloys at lower cost.

The copper suitable for use referred to herein as "oxygen-free copper" is readily recognizable by those skilled in the art as meaning a high purity copper which is substantially entirely free of oxygen by virtue of its having been processed by any of the known methods suitable for the purpose. Although electrolytic copper which has been processed in a reducing atmosphere such as "OFHC" brand copper provides excellent results, copper prepared in an inert atmosphere or in a vacuum or by any other suitable means as processing with carbon may also be used. Copper treated with chemical deoxidizers such as phosphorus and the like wherein the scavenging substance remains in the copper as an oxygen-containing compound or complex though sometimes erroneously re-

ferred to as "oxygen-free copper" is not satisfactory for use in making the wrought copper-titanium alloys herein disclosed.

The titanium content of the cast material suitable for use in making the wrought copper-titanium alloys comprising the present invention may be varied between 1 and 6% by weight, the lower limit representing the minimum titanium which must be present for any appreciable age-hardening to occur, whereas the upper limit represents approximately the maximum solid solubility of titanium in oxygen-free high purity copper which is found to occur at about 900° C. With the use of at least 3% titanium, minimum tensile strength values of 180,000 p.s.i. may be readily obtained in the wrought alloy upon employing appropriate working and heating cycles, while near the upper limit of titanium content the tensile strength approaches 220,000 p.s.i. For providing the most desirable combination of properties of the wrought material suitable for most applications, however, it is preferred to use from 3.8 to 4.3% titanium whereby cold drawn wire having a minimum tensile strength of 200,000 p.s.i. and other desirable mechanical properties including a minimum elongation of 1% and a 180,000 p.s.i. yield strength may be readily obtained after appropriate age hardening heat treatment of the worked material. Slight overaging of the alloys during precipitation heat treatment may be utilized to improve elongation and electrical conductivity with only a relatively small decrease in tensile strength.

For preparing castings suitable for use in making the high strength wrought alloys mentioned above, the titanium may be added to the oxygen-free copper as good quality titanium metal sponge, a copper-titanium master alloy, or in any other suitable form of satisfactory purity. It is essential that oxygen be excluded throughout the melting, alloying and casting procedures. In general practice, the initially oxygen-free copper protected by an inert gas such as helium or argon is first melted at 1200-1400° C. in a graphite crucible and the desired amount of titanium is then added allowing for usual titanium losses. The melt is then stirred with a graphite rod and, after a short holding period, the alloy is cast while still protected by the inert gas. A holding period of less than 1/2 hour at the designated temperature is usually sufficient to effect complete dissolution of the titanium whereby homogeneous castings which are free of porosity and have good surface characteristics are consistently obtained. Large alloy castings, such as commercial size wirebars, containing up to 6% titanium are found to be free of inclusions as determined by microscopic examination of their crystal structures.

Preheating of the castings to about 800 to 900° C. prior to hot working the alloy and subsequent solution annealing operations should be carried out in a protective atmosphere to protect the alloys from oxidation at the elevated temperatures. Heat treating involving the use of temperatures appreciably below 600° C. may be performed, if desired, in the absence of such precautionary measures to exclude air since relatively little, if any, oxidation occurs at the lower temperatures during the time interval generally involved.

The improved hot workability of the oxygen-free copper-titanium alloys compared to similar alloys all processed under oxygen-excluding conditions is readily seen from the appearance of the hot rolled bars shown in Fig. 1 wherein bar A consists of an alloy prepared with initially oxygen-free high purity copper (OFHC brand) containing 4.3% titanium; bar B is an alloy consisting of electrolytic tough pitch copper containing 4.5% titanium; and bar C is an alloy of phosphorus deoxidized copper containing 4.1% titanium. In each case, 1" diameter castings were preheated to 900° C. and hot rolled in a rod mill. As is evident, bars B and C show marked susceptibility to brittleness and fractured severely on hot working as evidenced by their appearance after either

the first or second pass (20-30% reduction). At the same stage of working, however, bar A shows no sign whatever of cracking. In fact similar specimens were found to be hot workable with reductions up to 65-85% without any indications of failure. It will be appreciated that this extent of working permits the desired complete deformation of the cast structure in the initial hot working step. A fourth bar (not shown) consisting of fire refined copper alloyed with 4.2% titanium completely disintegrated upon hot working during the first pass involving only a 20% reduction. Microscopic examination of each of the fractured samples revealed a great number of inclusions accumulated in each of the alloys excepting the oxygen-free copper-titanium alloy which was substantially free of inclusions. It is readily apparent from the foregoing that the initial oxygen content of either fire refined or electrolytic tough pitch copper which usually ranges from .03 to .05% markedly impairs the hot workability of castings alloyed with the designated amounts of titanium. Interestingly enough, when the copper is chemically deoxidized as in the case of the phosphorus deoxidized specimen (bar C), the alloys made thereof with titanium actually possess rather poor hot workability.

For best results the alloys of this invention are preferably hot worked in the red heat i.e. between 700 and 900° C. particularly when the titanium content exceeds 3%, but care must be taken to avoid heating much above 900° C. to preclude the formation of any liquid phase which would render the alloys hot-short.

In addition to the highly improved hot-workability of the present alloys, they further possess excellent cold working properties. It has been found that all these alloys, when uniformly recrystallized in the course of solution heat treatment to effect a complete dissolution of the titanium, may be cold worked very satisfactorily. Final reductions of more than 90% may be applied without overworking the alloys. It is preferred, however, to start the initial cold working with smaller reductions of about 30-50% utilizing solution anneals between working cycles to obtain uniform grain size. By way of illustration, hot rolled rods solution annealed at 900° C. may be initially cold rolled with about 40% reduction. After resolution annealing the material may then be further cold rolled with about 50% reduction, after which successive solution annealing and cold rolling may again be performed with up to a final cold reduction of about 94% without failure or any indications of an over-worked condition. By contrast, the other copper-titanium alloys of the type shown in Fig. 1 containing comparable amounts of titanium become embrittled rather rapidly thereby making the fabrication of the material as well as the development of any comparable combination of properties exceedingly difficult.

Although solution heat treatment temperatures between 850 to slightly over 900° C. may be employed, it is preferred to solution anneal the alloys of oxygen-free copper-titanium under non-oxidizing conditions at about 900° C. at which temperature the maximum solid solubility of titanium in oxygen-free copper occurs. The time required to effect complete solubilization of the titanium may be varied depending primarily upon the titanium content of the alloy and the solution annealing temperature employed. It has been found that two hours at 900° C. is generally conducive to best results though somewhat longer or shorter periods may be actually used.

In making the wrought alloys in accordance with the present invention, the preferred sequence of processing steps comprises preheating the cast material to about 900° C., hot working preferably in the red heat, solution annealing, quenching, cold working to the extent required with intermediate solution annealings if necessary and subsequently precipitation hardening the worked material. It should be understood, however, that other methods for producing the wrought alloys may also be

employed. For example, the castings may be cold rolled without initial hot rolling as by solution heat treating the cast material, say for 2 hours at 900° C., quenching in water and then directly cold rolling with about 50% reduction. The solution heat treatment and cold working cycle may be repeated to the extent required after which the alloy is subjected to appropriate age hardening. Then too, following final cold reduction, an additional solution annealing step may be used immediately prior to precipitation heat treatment of the material whereby the aging characteristics of the resulting alloy are modified to the extent that a higher aging temperature is usually required to produce maximum hardness.

The effect of age hardening at various temperatures upon tensile strength of the alloys having from 0.2 to 5.8% titanium is indicated in the diagram shown as Fig. 2. In each of the alloys there indicated by the various curves, the castings (1.3" diameter bars) were hot and cold rolled into 0.203" diameter rod with two intermediate solution anneals. The 0.203" diameter rod was then again solution annealed at 900° C. for 2 hours, quenched in water and cold drawn to 0.081" diameter wire with an 84% final cold reduction. The tensile strengths shown in the diagram were determined after heating the wire specimens thus obtained for two hours at various temperatures indicated on the abscissa. It will be seen from Fig. 2, that at 0.72% or less titanium,

of titanium following precipitation hardening of the samples for 2 hours at 400° C. are shown in the diagrams comprising Figs. 3 and 4. Prior to the specified heat treatment the processing of the castings (1.3" diameter bars) included preheating and hot working the material to 0.285" diameter rod, solution annealing at 900° C. for 2 hours, quenching in water, cold working to .203" diameter rod, again solution annealing at 900° C. for 2 hours and finally cold drawing to .081" diameter wire. 10 It will be seen from Fig. 3 that a minimum tensile strength of 200,000 p.s.i. is obtainable with the alloys above 3.8% titanium and together with the other properties including hardness (Fig. 4) it will be readily apparent that the alloys having 3.8 to 4.3% titanium comprise especially 15 suitable materials where strength, hardness, elongation and electrical conductivity are important factors. While possessing strength not exceeded by any other copper base alloys, the compositions of this invention unlike other copper-titanium alloys are characterized by excellent workability which greatly simplifies processing and fabrication procedures and makes available an excellent wrought alloy for various applications.

20 The following specific examples are given to more fully illustrate the properties of the copper base alloys of this invention:

#### Example 1

An oxygen-free copper of the following typical analysis

| S, percent | Pb, percent | Sb, percent | Bi, percent | Sn, percent | Fe, percent | Ni, percent | Mn, percent | O <sub>2</sub> , percent |
|------------|-------------|-------------|-------------|-------------|-------------|-------------|-------------|--------------------------|
| .002       | .0003       | <.0005      | <.0001      | <.0001      | .0005       | .0006       | <.00005     | <.0002                   |

little or no age hardening or increase in tensile strength occurs; the effect is greatest approximately between 3.0 to 4.3%, and at 5.8% titanium the effect of precipitation hardening is appreciably reduced.

Although temperatures between 300 and 600° C. may be used in the precipitation heat treatment or age hardening of the alloys containing from 1 to 6% titanium, the preferred temperature range is 350 to 450° C. with maximum age-hardening being obtained between 375 and 425 and especially at about 400° C. The time required may obviously be varied depending upon the temperature employed, said temperature being largely determined by the previous treatment of the material and by the specific property or combination of properties deemed most pertinent for the intended application of the wrought alloy. For developing maximum tensile strengths in the case of cold drawn wire, age hardening the worked material for about 2 hours at about 400° C. is conducive to best results. By extending the precipitation heat treatment at the same temperature, however, to from 3 to 5 hours or even longer, ductility and electrical conductivity is appreciably improved with only relatively slight reduction in the maximum tensile strength. Where increased ductility and conductivity are of principal importance, the material may be processed more rapidly by raising the precipitation heat treating temperature say to about 450° C. whereby the treatment time is reduced to about 2 hours in the usual case.

For precipitation heat treatment of cold rolled sheet, the heat treatment temperature may also be varied, preferably between 350 and 450° C. with maximum tensile strength being usually obtained in about 2 hours at 375 to 400° C. Since the extent of previous cold working affects the precipitation hardening characteristics in that the more extensively worked material requires a slightly lower temperature compared to material subjected to relatively less working, the temperature and time conducive to best results must be selected accordingly.

Tensile strength, elongation, electrical conductivity and hardness values of the alloys containing varying amounts

was used in making the castings employed in making the wrought materials herein described. By way of illustration, a 4 x 4" wirebar weighing 300 pounds was prepared by melting the copper initially in a CO atmosphere. 40 When the temperature reached between 1200 and 1400° C. the protective gas was changed to argon to preclude reaction with titanium after which sufficient titanium in the form of a 28% titanium 72% copper master alloy was added to provide a 4.5 titanium content (calculated). After stirring with a graphite rod, the melt was held at 1250° C. for an additional 15 minutes after which the alloy was cast in a water-cooled steel mold under argon gas. The casting was free of inclusions and analysis of the bottom and top sections of the bar analyzed 4.30% Ti indicating that the retained alloying metal was evenly dispersed throughout the bar and relatively little titanium was lost in preparation of the casting.

45 Smaller castings as 1 x 14" round castings weighing about 3 pounds were similarly prepared containing varying amounts of titanium ranging from an actual content of from 0.2 to 7.3%. The melting, alloying and casting procedure was substantially the same as described above excepting that the alloys were cast in a copper mold.

#### Example 2

For determining the solvus and liquidus lines of the binary system consisting of oxygen-free copper and titanium, samples prepared as described in the preceding example were microscopically studied after heating to various temperatures for from 2 to 20 hours. Up to 6.07% Ti, hot and cold rolled rods of 0.285" diameter were used; the alloys of higher Ti content being subject to fracturing during hot rolling were studied in cast condition. The specimens were first heated for 20 hours at 885° C. and at 900° C., quenched in water and then reheated at various temperatures above and below 900° C.

70 The maximum solubility of titanium was found to occur at 900° C., the amount being close to 6%; at higher titanium contents, a hard undissolved phase consisting of Cu<sub>3</sub>Ti persisted whereas below 6% only the alpha phase

was obtainable upon appropriate heat treatment. The solid solubility limit of titanium below 575° C. was found to be between 0.3 and 0.7%, and at room temperature it is less than 0.5%; very close to 2.9% is soluble at 750° C., about 2.9% at 800° C. and close to 5% at 850° C. The maximum solid solubility limit was further indicated by marked brittleness of the alloys upon hot or cold working containing in excess of 6% titanium whereas those containing within the maximum solid solubility amount could be worked upon appropriate solution annealing without difficulty.

#### Example 3

A sample from a 4 x 4 x 60 inch wirebar containing 4.3% Ti which was preheated in a partially reducing atmosphere for 90 minutes to a temperature between 870 to 900° C. was forged into a 2 x 2" square with 50% reduction. Microscopic examination of the sample showed that the cast crystals in the center of the bar were not completely deformed indicating the need for working more than 50% to induce a homogeneous recrystallized structure. When worked to 65% reduction or higher, a uniformly recrystallized structure of the forging consisting of alpha plus Cu<sub>3</sub>Ti precipitate in the alpha-grain boundaries was obtained.

#### Example 4

The effect of the amount of cold working on some properties of the subsequently age-hardened alloy is illustrated by the following: a 1" diameter casting containing 4.3% Ti prepared as described in Example 1 was hot worked to 0.25" diameter and cold worked to 0.203" wire with intermediate solution annealing. The 0.203" wire, after being solution annealed at 900° C. for 2 hours and cold drawn to different final reductions in area, was then precipitation heat treated for 2 hours at 375-400° C. The tensile strength and elongation values obtained are as follows:

| Percent Cold Rolling | Tensile Strength (p.s.i.) | Elongation (percent in 2") |
|----------------------|---------------------------|----------------------------|
| 20                   | 120,000                   | 18.0                       |
| 35                   | 134,800                   | 10.4                       |
| 57                   | 165,000                   | 2.8                        |
| 66                   | 177,000                   | 2.2                        |
| 74                   | 182,000                   | 1.0                        |
| 78                   | 190,000                   | 0                          |
| 84                   | 208,000                   | 0                          |
| 92                   | 210,000                   | 0                          |

It will be seen from the above that the tensile strength and elongation properties vary appreciably with the amount of final cold reduction applied prior to the age hardening step.

#### Example 5

As seen from the preceding example, increasing the amount of cold working between solution annealing and precipitation heat treatment results in an increase in tensile strength and a lowering of the ductility of the alloy. Though the alloys and particularly the preferred compositions containing 3.8 to 4.3% Ti exhibit excellent hot and cold workability and extremely high tensile strength, the elongation after age hardening for 2 hours at the optimum temperatures for maximum strength is usually very low and often not even a measurable amount. As previously stated, however, elongation as well as other properties such as electrical conductivity may be improved by overaging the alloy.

The results achieved by extending the time of treatment at a given age hardening temperature is illustrated by the following data obtained on a 4.3% Ti alloy processed by hot and cold working with intermediate solution anneals and with a final cold reduction of 84% to provide 0.081" diameter wire. Specimens of the wire were heat treated at 375° C. for the indicated periods and then tested for

tensile strength, elongation and electrical conductivity. The values obtained are listed as follows:

| Time (hrs.) at 375° C. | Tensile Strength (p.s.i.) | Elongation (percent in 2") | Electrical Conductivity (percent) |
|------------------------|---------------------------|----------------------------|-----------------------------------|
| 0                      | 161,000                   | 1                          | 3                                 |
| 0.5                    | 167,000                   | 0                          | 5                                 |
| 1                      | 176,000                   | 0                          | 6                                 |
| 2                      | 209,000                   | 0                          | 7                                 |
| 3                      | 209,400                   | 0                          | 7                                 |
| 4                      | 210,200                   | 0                          | 7                                 |
| 5                      | 205,500                   | 1.0                        | 10                                |
| 22                     | 203,500                   | 1.0                        | 15                                |

Specimens heat treated at 400° C. for the specified periods of time possessed the following properties:

| Time (hrs.) at 400° C. | Tensile Strength (p.s.i.) | Elongation (percent in 2") | Electrical Conductivity (percent) |
|------------------------|---------------------------|----------------------------|-----------------------------------|
| 0                      | 161,000                   | 1                          | 3                                 |
| 0.5                    | 190,000                   | 0                          | 4                                 |
| 1                      | 203,000                   | 0                          | 7                                 |
| 2                      | 210,000                   | 0.4                        | 10                                |
| 3                      | 205,500                   | 1                          | 11                                |
| 4                      | 202,000                   | 1                          | 11                                |
| 5                      | 201,000                   | 1                          | 15                                |
| 17                     | 190,000                   | 2                          | 18                                |

It will be apparent from the above that at 375° C. the elongation of the 4.3% Ti alloy may be improved to 1% by extending the age hardening time to a minimum of 5 hours. During such treatment the electrical conductivity is also improved and the tensile strength is decreased only slightly.

By age hardening at 400° C., it will be seen that the time required to improve elongation of the same alloy is appreciably reduced. At this temperature a minimum elongation of 1% and improvement in conductivity to 10% with only a slight decrease in tensile strength is obtained within 3 to 5 hours.

#### Example 6

Specimens of the same alloy prepared as described in the preceding example subjected to heat treatment at 450° C. for 2 hours were lowered in tensile strength to 180,000 p.s.i. but elongation was increased to 3.6% and electrical conductivity to 20% by this treatment. The yield strength of the 84% cold drawn 0.081" diameter wire determined after the 2-hour heat treatment at 450° C. was 170,000 p.s.i., after 5 hours at 375° C. it was 194,000; and 180,000 p.s.i. after 4 hours at 400° C.

#### Example 7

Alloys containing 3.0 and 4.3% Ti respectively cold rolled to 0.285" diameter rods were solution annealed for 2 hours at 900° C., quenched and then age hardened for 2 hours at various temperatures to determine the effect of precipitation heat treatment on the solution annealed material. Maximum precipitation hardening for both alloys resulting in hardness values ranging from 255 to 290 V.P.N. was found to occur at 450-500° C. By heating specimens of the solution annealed rod material at 475° C. for varying periods of time ranging from 0.5 to 50 hours to observe the effect of time, it was found that approximate maximum hardening of the material was obtained within an hour with only a small increase up to 4 hours. Heating over 16 hours was found to slowly decrease the hardness.

In the case of 0.182" diameter wire made with a 4.3% Ti alloy, precipitation heat treatment for 3 hours at 475° C. after solution annealing yielded a material of 133,600 p.s.i. tensile strength and 16.8% elongation.

#### Example 8

Sheet material of 0.10 and 0.30" thickness was made from 4.3% Ti castings by hot rolling on flat rolls with

minimum reductions of 65% and as much as 85% and by cold rolling with intermediate solution annealing. After a final solution annealing for 3 hours at 900° C., the sheets were cold rolled with 85 and 94% reductions and then age hardened. In the case of 0.045" thickness sheet made from the 0.30" sheet cold worked to 85% final reduction, optimum strength of 195,000 p.s.i. with 1% elongation and a yield strength of 180,000 p.s.i. was obtained in 2 hours at 375° C. and upon increasing the age hardening temperature to 400° C., at the end of 2 hours the tensile strength was reduced to 170,000 p.s.i. but the elongation increased to 2%. The 0.10 sheet material similarly solution annealed at 900° C. for 3 hours after cold working to a final reduction of 94% to provide sheet of 0.019" thickness upon age hardening for 2 hours at 375° C. yielded a maximum tensile strength of 203,000 p.s.i., but the elongation was nil. By extending the age hardening time to 4 hours at the same temperature, however, material having a tensile strength of 195,000 p.s.i., elongation of 1% and yield strength of 189,000 p.s.i. was obtained. By increasing the age hardening temperature to 400° C., good properties including tensile strength of 190,000 p.s.i., minimum elongation of 1% and yield strength of 165,000 p.s.i. were obtained in only 2 hours.

It is apparent that many differing embodiments of this invention may be made without departing from the spirit and scope thereof and it is not intended to be limited except as indicated in the appended claims.

I claim:

1. In the process of making copper-titanium alloys, the improvement comprising the steps of alloying initially oxygen-free copper under oxygen excluding conditions with sufficient titanium to provide a titanium content of from 1 to 6% by weight in the resulting cast alloy, pre-heating said cast alloy and hot working the same to ef-

fect a reduction in cross-sectional area of at least 50%.

2. In the process of making copper-titanium alloys, the improvement comprising the steps of alloying initially oxygen-free copper under oxygen-excluding conditions with sufficient titanium to provide a titanium content of from 3.8 to 4.3% by weight in the resulting cast alloy, preheating said cast alloy and hot working the same to effect a reduction in cross-sectional area of at least 50%.

3. The process of making wrought copper-titanium alloys which comprises the steps of alloying initially oxygen-free copper under oxygen-excluding conditions with sufficient titanium to provide a titanium content of from 1 to 6% in the resulting cast alloy, preheating said cast alloy and hot working the same to effect a reduction in cross-sectional area of at least 50%, solution annealing the hot worked material at about 850 to 900° C., quenching, cold working and thereafter age hardening the alloy at a temperature between 300 and 600° C.

4. The process of claim 3 wherein the titanium content of the cast alloy is adjusted to form 3.8 to 4.3% by weight and the age hardening step is carried out at a temperature ranging from 350 to 450° C.

#### References Cited in the file of this patent

#### UNITED STATES PATENTS

|           |                |               |
|-----------|----------------|---------------|
| 935,863   | Rossi          | Oct. 5, 1909  |
| 2,201,555 | Carson         | May 21, 1940  |
| 2,783,143 | Johnson et al. | Feb. 26, 1957 |
| 2,842,438 | Saarivirta     | July 8, 1958  |

#### OTHER REFERENCES

Journal of Metals, volume 4, July 1952, page 766, "Titanium Copper Binary Phase Diagram," by Joukainen et al.

35 Metals Handbook, 1948, edition, by American Society for Metals, page 880.